

## UNITED STATES PATENT OFFICE

1,941,202

## ALLOY STEEL

Henry A. De Fries, Albany, N. Y., assignor to  
 Ludlum Steel Company, Watervliet, N. Y., a  
 corporation of New Jersey

No Drawing. Application March 29, 1929  
 Serial No. 351,119

3 Claims. (Cl. 75—1)

My invention relates to improvements in those alloy steels containing chromium in sufficient quantity to render them substantially rustless or stainless, whereby they are more easily forged, 5 machined, or ground, and whereby their non-corrosive properties are improved.

Alloy steels containing up to 30% of chromium, and particularly those containing from 12% to 10 20%, are widely used because of their high resistance to corrosion although considerable difficulty is experienced in the forging, machining and grinding thereof.

It is well known that a comparatively high sulphur content improves the forgeability of ordinary steels, but the presence of this element in so-called stainless steels, in an amount sufficient 15 to appreciably affect the workability thereof, is extremely detrimental to if not destructive of the very property—stainlessness—which prompts 20 the use of such steels.

I find that alloy steels having a high resistance to corrosion and containing up to 30% of chromium may be rendered comparatively easy to forge, machine and grind, and that their corrosion resisting characteristics are not impaired 25 by the presence of from 0.10% to 0.50% of sulphur provided a small amount of copper, say from 0.20% to 1.20%, is also present. The copper not only neutralizes the detrimental effect of the 30 sulphur upon the stainless properties of the steel but materially improves these properties.

The following alloy steel, for example, has high resistance to corrosion, will flow readily in forging dies, can be easily machined, and can be 35 ground more readily than regular carbon steel:

|            |               |
|------------|---------------|
| Carbon     | 0.07%—0.12%   |
| Manganese  | 0.30%—0.50%   |
| Silicon    | 0.30%—0.70%   |
| Chromium   | 15.00%—16.00% |
| Copper     | 0.50%—0.75%   |
| Sulphur    | 0.25%—0.35%   |
| Phosphorus | 0.025 max.    |

In making a steel of this character, I prefer 45 to add the copper and sulphur together in the form of copper matte, an intermediate product

of the copper smelting process and an intermetallic compound conforming to the formula Cu<sub>2</sub>SFeS. This may be added to the molten alloy either in the furnace or in the ladle, and in lump or granular form. From one to three 60 pounds of copper matte per hundred pounds of steel will greatly improve its forgeability and machineability and at the same time, increase its resistance to corrosion.

In the claims I have used the expression "the 65 remainder being iron". This is to be understood as including iron and elements such as carbon, silicon, manganese, and phosphorus within the limits usually encountered in steel making practice.

What I claim is—

1. A steel alloy containing as essential ingredients chromium from 1% to 30%, copper from 0.20% to 1.20%, and sulphur from 0.10% to 0.50%; the remainder being iron; said alloy 75 having a resistance to corrosion comparable to an alloy steel containing chromium in the above range with sulphur low and under 0.10%, and being characterized by its easy machinability and forgeability.

2. A steel alloy containing as essential ingredients chromium from 12% to 20%, copper from 0.20% to 1.20%, and sulphur from 0.10% to 0.50%; the remainder being iron; said alloy 85 having a resistance to corrosion comparable to an alloy steel containing chromium in the above range with sulphur low and under 0.10%, and being characterized by its easy machinability and forgeability.

3. A steel alloy containing as essential alloying ingredients chromium from 1% to 30%, at least 90 0.10% of sulphur and at least 0.20% of copper; the total copper and sulphur being under 2% with the copper at least twice the sulphur; the remainder being iron; said alloy having a resistance to corrosion comparable to an alloy steel containing chromium in the above range with sulphur low and under 0.10%, and being characterized by its easy machineability and forgeability.

HENRY A. DE FRIES.